

May 31, 1932.

F. W. ABRAMS

1,860,798

METHOD FOR MAKING SOAP OIL COMPOSITIONS

Filed July 14, 1926



FRANK W. ABRAMS Inventor

By Attorney, *C. H. Straw*

Patented May 31, 1932

1,860,798

# UNITED STATES PATENT OFFICE

FRANK W. ABRAMS, OF ELIZABETH, NEW JERSEY, ASSIGNOR TO STANDARD OIL DEVELOPMENT COMPANY, A CORPORATION OF DELAWARE

## METHOD FOR MAKING SOAP-OIL COMPOSITIONS

Application filed July 14, 1926. Serial No. 122,348.

This invention relates to improvements in the manufacture of hydrocarbon oil compositions containing soap. In accordance with the invention, a soap is associated with the oil under such conditions that a fluid product is formed in which the soap appears to exist as a colloid. The method will be fully understood from the following description, taken in connection with the accompanying drawing, in which the figure is a diagrammatic side elevation partly in section, showing one suitable form of apparatus.

As illustrative of the invention, the manufacture of a soap-containing lubricating oil will be described. Mineral oil of about 75 seconds Saybolt viscosity at 212° F. is supplied from tank 1 through pipe 2, pump 3 and pipe 4 to the agitator 5. Valves 6, 7, and 8 are open and valves 9, 10, 11 and 26 are closed while the agitator is being charged. When this is completed the oil is drawn by pump 3 through pipe 12 connected to the bottom of the agitator and through pipe 13 to a heater 14, preferably a continuous coil heated by flue 15 gases. From the heater 14 the oil passes through pipe 15 and is discharged below the surface of the oil in agitator 5.

A draft tube 16 is arranged in the central portion of the agitator, and a stirrer 17 of the propeller type operates in the lower portion of the draft tube. The draft tube terminates just below the surface of the liquid whereby violent surface agitation is obtained upon actuation of the stirrer. During the earlier stages of the operation the stirrer should be rotated so as to cause an upward flow of oil through the draft tube. If rotated in a reverse direction, air is drawn in and may discolor the oil.

When the temperature of the oil in the agitator has reached about 120° F., the calculated amount of oleic acid (elaine or red oil) is drawn from a tank 18 through pipe 19 and is fed into the agitator 5, wherein it is thoroughly mixed with the oil. When the mixture of oil and oleic acid has reached a temperature of about 180° F., the calculated amount of a 25% aqueous solution of sodium hydroxid, required to substantially neutralize the oleic acid, is drawn from tank 20 by

pipe 21 to the agitator 5. The soap formed by the neutralization may, for example, constitute about 0.17% by weight of the composition and will in most cases be less than 0.5%. The agitation, circulation and heating, as described, are continued throughout the operations referred to.

When a temperature of about 220° F. is reached, steam is injected over the surface of the oil in the agitator through steam inlet 22, in order to exclude air. A ventilator 23 is provided at the top of the agitator and serves to allow the escape of excess steam, either injected or formed from water that may be present in the oil.

At temperatures around 212° F. foam ordinarily begins to form. The direction of rotation of the stirrer is now reversed so as to destroy the foam by drawing it under the surface of the oil. Since the temperature of the agitator is now high enough to permit the maintenance of an atmosphere of steam, no substantial amount of air is drawn into the oil.

The amount of heat supplied in heater 14 should be so regulated that the oil in the agitator is brought gradually up to a temperature not generally exceeding 10° F. below the flash point of the oil in from 10 to 15 hours. At the end of this period it will be found that the reaction between the oleic acid and sodium hydroxid is completed and that substantially all water has been removed from the composition. The circulation and agitation are continued for a short time to insure thorough mixing and to expel the last traces of water.

The hot contents of the agitator is then pumped through pipe 12 to cooler 24. The composition remaining in the heater 14 and the pipe lines is also pumped to the cooler, a by-pass 25 being provided for this purpose. During the pumping out of the agitator, valves 26, 7, and 11 are open and valves 6, 8, 9, and 10 are closed. The valves 9, and 9' in the by-pass 25, as well as valves 7 and 11 in the main lines, are opened when the heater and pipe lines are to be pumped out. During this operation valves 6, 8, 10 and 26 are

closed. The cooled product is drawn off through pipe 27 to a storage tank 28.

It is important that the composition be cooled rapidly, as otherwise gel formation is likely to occur. Rapid cooling, coupled with considerable agitation, such as may be effected in a long pipe coil with numerous bends, is desirable. Vigorous agitation without positive cooling will also serve in many cases to prevent the formation of a gel. However, rapid cooling is desirable through the temperature range (in the process described about 400-150° F.) in which the gel is likely to appear. If the gel does not form within this temperature range, the composition will be stable; that is, it will show no separation of soap even after long standing, but will remain a clear, apparently homogeneous liquid. The invention is particularly adapted for the preparation of oils containing soap in amount which will not increase greatly the viscosity of the oil; the soap being present in amount and physical condition adapted to improve the film-maintaining property of the oil.

While it is desirable to form a soap in the body of oil, it may be added in other ways, for example, preformed, as a solid or in water or alcohol solution.

The invention is not limited to the use of the special materials, proportions, and operating conditions described. Various changes and alternative arrangements may be made within the scope of the appended claims, in which it is my intention to claim all novelty inherent in the invention as broadly as the prior art permits.

I claim:

1. Method of manufacturing a hydrocarbon oil composition containing soap, comprising circulating the oil through a cycle including an agitating zone and a heating zone, distributing a soap in the oil, and rapidly cooling the composition through the temperature range in which gel formation would otherwise take place.

2. The method of manufacturing a hydrocarbon oil composition containing soap, which comprises maintaining a body of hydrocarbon oil, continuously abstracting a part thereof, passing said part through a heating zone and returning same to said body, distributing a soap in said oil and rapidly cooling the oil and distributed soap through the temperature range in which gel formation would otherwise take place.

3. The method of manufacturing a hydrocarbon oil composition containing soap, which comprises maintaining a body of lubricating oil, heating the oil, incorporating a soap therein and stirring said body of oil containing soap upwardly, continuing the heating of said body until the temperature of the same is in excess of 212° F., forming a blanket of steam over the surface of said body when

the temperature is in excess of 212° F., and after the formation of said blanket stirring the liquid downwardly sufficiently rapidly to draw surface matter into the liquid.

4. The method of manufacturing a hydrocarbon oil composition containing soap, which comprises incorporating the soap in the oil, heating the mixture to a temperature approximating the condensing point of steam, disposing the heated mixture in a body the upper surface of which is exposed to the air, agitating the mixture, heating the mixture until a temperature above the condensation point of steam is reached, disposing an atmosphere of steam upon the surface of the body, and stirring the body of mixture downwardly with violent surface agitation in the atmosphere of steam.

5. The method of manufacturing a hydrocarbon oil composition containing soap, which comprises incorporating the soap in the oil, heating the mixture to a temperature above the condensation point of steam, disposing the mixture in a body, maintaining an atmosphere of steam upon the surface of the body, and stirring the mixture by drawing the liquid downwardly from the surface in a tubular zone of the body with violent surface agitation.

FRANK W. ABRAMS. 95

100

105

110

115

120

125

130